

3,233,960

## DYEING AND PRINTING OF POLYOLEFINS

Bruno Lonardo, Milan, Italy, assignor to Aziende Colori Nazionali Affini—ACNA S.p.A., Milan, Italy  
No Drawing. Filed May 10, 1963, Ser. No. 279,601  
Claims priority, application Italy, May 15, 1962,  
9,721/62, 9,722/62  
9 Claims. (Cl. 8—34)

The present invention relates to a method for the application of vat dyestuffs in the dyeing and printing of polyolefins.

More particularly, the present invention relates to a method for dyeing and printing of vat dyestuffs on a polyolefin, which method comprises:

(a) Impregnating a polyolefin with either a solution of a vat dyestuff in leuco form or a dispersion of a vat dyestuff;

(b) Thermally treating the impregnated polyolefin;

(c) Where a vat dyestuff dispersion is used, then subjecting the thus thermally treated, impregnated polyolefin to reducing conditions to reduce the dyestuff to the leuco form; and

(d) Subjecting the impregnated polyolefin to oxidation while contemporaneously soaping such polyolefin with a soap solution at its boiling temperature.

The present invention also relates to the polyolefin materials dyed according to the above mentioned method.

It is well known that articles made from synthetic material obtained by the polymerization of hydrocarbons containing no polar groups, e.g., ethylene, propylene, methylpentene-1, etc., are most difficult to dye by the dyestuffs and methods conventionally employed because of their lack of affinity for such dyestuffs.

Such incompatibility to dyeing and the unsatisfactory results obtained have led to three attempted solutions to the problem:

(1) Dyeing in mass, using pigments of the synthetic material before shaping or spinning; this has definite disadvantages because it is necessary that the semi-finished material be produced in the final dye;

(2) A previous partial modification of the material, comprising adding, during the shaping and spinning operation, dyeable substances to the polymer which permits the dyeing of the shaped articles; this technique is disadvantageous in that it is comparatively expensive, yet the final product may not completely be homogeneous.

(3) Substantial modification of either the entire material during the preparation of the polymer, or its surface after it has been shaped, comprising introducing into the polymer molecule atoms other than C and H, or introducing functional groups different from the paraffinic groups (contemplating also the formation of copolymers), in order to render the material dyeable; this technique has the drawback that the modification of the polymer molecule may lead to a change of the characteristics of the product.

The present invention goes beyond the solutions described in foregoing items (1), (2) and (3), since it relates only to non-modified polymers, and to the non-modified polymer portions in the physical or mechanical mixtures together with other materials.

Particularly as regards polypropylene, a very high incompatibility has been shown with respect to dyeing carried out using conventional dyestuffs and dyeing methods.

Results having a practical interest, although very restricted, have been hitherto obtained by the application of vat dyestuffs in dyeing.

The application of vat dyestuffs on textile materials made up of polyolefins, particularly polypropylene, may be carried out for instance according to the following

method: Reduction of the dyestuff in a main vat bath using the sodium salt of the sulforicinoleic acid, sodium hydroxide and sodium hydrosulfite in those amounts and under those conditions generally used for cotton dyeing; preparation of the bath and dyeing using the required amounts of main vat bath, water, and the conventional additional amounts of sodium hydroxide and sodium hydrosulfite required; beginning the dyeing at about 150° C. and gradually adding ammonium acetate up to a total concentration of above 9 g./l. over a period of 15 to 20 minutes; gradually heating at about 45° C. and carrying on the dyeing at this temperature for about 30—40 minutes while maintaining the pH at between 9.5 and 10 and seeing that an excess of sodium hydrosulfite is always present; rinsing the material with cold water; soaping for 20—30 minutes at the boiling temperature using a solution containing 2 g./l. of an anionic detergent and between 1 and 2 cc. of 30% hydrogen peroxide; rinsing; and drying the material.

Dyes suggested for use in the above process include 1,2,5,6 - diphenyl - dithiazol - anthraquinone; dibromo - anthranthrone; isoviolanthrone; 4,4' - dimethyl - 6,6' - dichloro - thioindigo; 5,7,5',7' - tetrabromo - thioindigo; 4,4" - dibenzamido - anthraquinon-4,1',10,1" - diimido - anthranthrone; dibromo-dimethoxy-dibenzanthrone; 1,1', 4,5' - dibenzoyl - diamino - diantramide; 2,3',3,2" - tri-anthraquinol-1,4',1" - diimide; product of the alkaline condensation of 1',3,1',9-diimidoanthraquinonebenzanthrone (having respectively the following Color Indexes, C.I. 67300, 59105, 60010, 73360, 73065, 65225, 59830, 69015, 70800, 69525).

The dyeing process involves a penetration of the dyestuffs in the reduced state followed by fixation in the oxidized state of the dyestuffs in the surface pores of the material.

By dyeing according to this method and using appropriate concentrations of each of the above mentioned dyestuffs, materials are obtained having a very bright shade but with an intensity not greater than those which are  $\frac{1}{2}$  of the standard ECE intensity scale. It is clear that such a limitation of the dyeing capabilities severely limits the possible sales potential and marketing of the material. Further, the fastness to rubbing of the dyed materials thus obtained is very low, so that such dyed materials and articles are not suitable for use in home furnishings. Moreover the fastness to organic solvents is so low that dry washing of the colored material is impossible without completely affecting the dyeings. These drawbacks clearly adversely affect the marketing potential of the materials dyed by this technique.

There has now surprisingly been found a method by which it is possible to dye polyolefin materials using vat dyestuffs, whereby the dye product exhibits an intensity 1/1 in the ECE standard scale.

This method comprises:

(a) Impregnating a polyolefin with either a solution of a vat dyestuff in leuco form or a dispersion of a vat dyestuff;

(b) Thermally treating the impregnated polyolefin;

(c) Where a vat dyestuff dispersion is used, then subjecting the thus thermally treated, impregnated polyolefin to reducing conditions to reduce the dyestuff to the leuco form; and

(d) Subjecting the impregnated polyolefin to oxidation while contemporaneously soaping such polyolefin with a soap solution at its boiling temperature.

In accordance with one embodiment of this invention, a vat dyestuff in leuco form is applied to the polyolefin material, followed by a heat treatment and a subsequent reoxidation of the dyestuffs while on the material.

More particularly, this embodiment of the dyeing method of the present invention is characterized by the following successive steps:

(a) Impregnation of the polyolefinic material with a solution of the vat dyestuff in the leuco form, generally in the presence of additives;

(b) Heat treatment at about 125° C.;

(c) Oxidation in an oxidizing bath, preferably using hydrogen peroxide, while contemporaneously soaping the polyolefin with a soap solution at its boiling temperature.

Dyeing according to this embodiment is desirably carried out as follows:

Reduction of the dyestuffs in a main vat bath using NaOH and sodium hydrosulfite in such amounts and conditions as are generally employed for dyeing cotton; preparation of an impregnating bath by the addition of appropriate additives, e.g., those which facilitate the dyestuff penetration and levelling (e.g., diethyl tartrate) and also anionic dispersing agents (e.g., the sodium salt of the ligninsulfonic acid); dilution with water containing sodium hydroxide and sodium hydrosulfite to obtain the desired dyeing intensity; eventual thickening by means of conventional thickening agents; impregnation of the polyolefin material at from about 10°-60° C.; treatment in a hot air oven at 120-125° C. for a period of time varying from about 1 minute to 10 minutes; rinsing of the material with cold water; and simultaneously oxidizing and soaping using a solution at its boiling temperature for from about 20-30 minutes, which solution contains an anionic detergent, for instance, the sodium salt of oleyl-methyl-taurinic acid (conc. ~2 g./l.) or the sodium salt of oleic acid (conc. 2 g./l.) along with 1 to 2 cc. per liter of 30% hydrogen peroxide; rinsing and drying of the thus dyed material.

In accordance with another embodiment of the present invention, vat dyestuffs in the dispersed state are applied to polyolefin material, such dyestuffs are then reduced to the leuco form and thereafter are reoxidized while on the material.

More particularly, this embodiment is characterized by the following successive steps:

(a) Impregnation of the polyolefin material with a dispersion of vat dyestuffs, desirably in the presence of additives;

(b) Thermal treatment at about 125° C.;

(c) Reduction of the dyestuff on the polyolefin material in a reducing bath; and

(d) Oxidation in an oxidizing bath, preferably with hydrogen peroxide with contemporaneous soaping treatment at the boiling temperature of the soap solution.

Preferably, this embodiment is carried out as follows:

Preparation of an impregnating bath by the use of the suitable amounts of water, vat dyestuffs (in the form of a paste or fine powder having particle sizes lower than about 1 micron) and anionic dispersing agents (for instance the sodium salt of ligninsulfonic acid or the sodium salt of the naphthalene-sulfonic acid or the sodium salt of the dinaphthylmethane-disulfonic acid); addition of appropriate additives e.g., diethyl tartrate, to facilitate dyestuff penetration and levelling; eventual thickening by the aid of conventional thickening agents; impregnation of the polyolefin material at from about 50-60° C.; treatment in a hot air oven at 120-125° C. for a period of time varying from about 1 minute to 10 minutes; reduction of the dyestuff on the material in an aqueous bath containing sodium hydroxide and sodium hydrosulfite while keeping the pH between 9.5 and 10 by gradual additions of ammonium acetate; this reduction occurring while the temperature is maintained at from about 50-60° C., and during a period of time of about 30 minutes; rinsing with cold water; soaping for 20-30 minutes with a solution at its boiling temperature, this solution containing an anionic detergent (for instance, the sodium salt of oleyl-methyl-taurinic acid or the sodium salt of oleic acid at a con-

centration of 2 g./l.) and one to two cc. per liter of 30% hydrogen peroxide; rinsing and drying of the material.

In accordance with either of the foregoing embodiments, suitable dyestuffs include anthraquinone, indigo, thioindigo, carbazole, benzathrone, anthranthrone, and the like, either in their simple form, or substituted, or condensed with one another.

By the method of this invention, it is possible to obtain articles made from polyolefins, particularly polypropylene, which are dyed at 1/1 intensity of the Standard ECE scale. This is made possible by the simultaneous use of high temperatures, dispersing agents, and additives, and, in one embodiment, dyestuffs consisting of particles of tiny size. The foregoing results in a remarkable penetration of the dyestuff into the material to be dyed.

The advantages of the present invention as compared to known dyeing methods are the following: a widening of the range of vat dyestuffs which are usable with polyolefins, and in particular on polypropylene; a remarkable increase in the intensities which may be obtained; fastnesses for the dyed articles which are at least equal to and are generally higher than those of articles dyed according to previously known methods; in particular, resistances to rubbing at 1/12 intensities are higher than those of articles dyed at 1/12 intensities according to previously known methods.

The dyestuffs utilized in the examples hereinafter have been found to be particularly suitable. However, other vat dyestuffs may also be employed according to the method of the invention.

The present invention is also directed to polyolefin materials, in particular polypropylene materials (such as fibers, films and other manufactured articles) which have been dyed according to the method of this invention.

By comparing the results of the dyeing obtained according to the method of the present invention with those obtainable according to the known methods, the advantages attained by the method of the present invention are clear.

Further, the method of this invention may be applied to molded articles. The variation to be effected for this use resides in a suitable regulation of the viscosity of the leuco-alkaline solution of the vat dyestuffs by thickening agents.

The following examples will further illustrate the invention. Examples 1-23 illustrate that embodiment of the invention wherein the dyestuff is applied as a solution and is in leuco form.

#### EXAMPLE 1

A sample of polypropylene fiber is impregnated (in a Foulard apparatus) in an aqueous bath at 60° C., containing 25 g./l. of brilliant green Romatrene FFB (C.I. 59825) reduced to leuco-alkaline compound with 42 g./l. of a 36 Bé. NaOH, 15 g./l. sodium hydrosulfite and 25 g./l. of the sodium salt of dinaphthyl-methane-disulfonic acid.

The impregnated material is treated for 6 minutes in a continuous polymerization reaction heated by hot air to 120-125° C., rinsed in cold water, soaped for 30 minutes with a solution at its boiling point, which solution contains the sodium salt of oleyl-methyltaurinic acid and an oxidizing agent, namely, 30% hydrogen peroxide (concentration=2 cc./l.), rinsed, and dried.

The fiber is dyed green with good uniformity and a 1/1 intensity according to the ECE Standard scales. It exhibits good general fastness and fastness to natural light of at least one point on 8 higher than that for a dyeing obtained on the same fiber using the same dyestuff reduced in a bath at 50° C. and a pH 9.5-10.

#### EXAMPLE 2

This example is similar to Example 1, however, there is added to the impregnating bath a suitable amount of additives to facilitate the penetration and the levelling, namely, 25 g./l. of diethyl tartrate, and also thickening

agents compatible with the bath, namely, Nafka rubber (concentration=10 g./l.).

The fiber is dyed green and has the same characteristics as that obtained in Example 1. It has, however, even a higher uniformity, a higher purity, and a brighter shade.

### EXAMPLES 3-17

By operating as described in Example 1, using the dyestuffs reported in Table 1; results and advantages similar to those mentioned in Example 1 are obtained.

Table 1

| Example Number | Dyestuff                        | Color Index | Shade        |
|----------------|---------------------------------|-------------|--------------|
| 3              | Tomantrene yellow GCN           | C.I. 67300  | Yellow.      |
| 4              | Golden yellow Romantrene FRK    | C.I. 59105  | Do.          |
| 5              | Brilliant pink Romantrene FR    | C.I. 73360  | Pink.        |
| 6              | Brilliant violet Romantrene F2R | C.I. 60010  | Violet.      |
| 7              | Bromoindigo 2BD                 | C.I. 73065  | Blue.        |
| 8              | Brilliant green Romantrene F2G  | C.I. 59830  | Green.       |
| 9              | Brown Romantrene FR             | C.I. 69015  | Brown.       |
| 10             | Brown Romantrene FBR            | C.I. 70800  | Do.          |
| 11             | Olive Romantrene FT             | C.I. 69525  | Olive.       |
| 12             | Yellow Romantrene F3RT          | C.I. 70805  | Yellow.      |
| 13             | Olive Romantrene FR             | C.I. 69005  | Olive.       |
| 14             | Blue Romantrene FRS             | C.I. 69800  | Blue.        |
| 15             | Blue Romantrene FGD             | C.I. 69810  | Do.          |
| 16             | Blue Romantrene FBC             | C.I. 69825  | Do.          |
| 17             | Dark blue Romantrene FBO        | C.I. 59800  | Blue marine. |

### EXAMPLE 18

By operating as described in Example 2 using each of the dyestuffs reported in Table 1, results are obtained which are similar to those reported in Example 2.

### EXAMPLE 19

By operating as described in each of Examples 1 and 3 to 17, but using samples of compact polypropylene and polyethylene sheets, similar results to those reported for Example 1 were obtained.

### EXAMPLE 20

By operating as described in each of Examples 2 and 18, but using samples of compact polypropylene sheet, results similar to those reported for Example 2 were obtained.

### EXAMPLE 21

On a fabric of polypropylene fiber a printing is made, using a paste prepared as described in Example 2, but using a higher amount of thickening agent (for instance 5-10 g./100 cc.).

The printed material thus obtained is finished as described in Example 1. Good printing results were obtained, as shown by good penetration, uniformity, and fastness and other characteristics similar to those for the articles dyed as described in Example 2.

### EXAMPLE 22

By proceeding according to the method described in Example 21, using each of the dyestuffs reported in Table 1, results similar to those specified in Example 21 were obtained.

### EXAMPLE 23

By proceeding as described in Example 22, but using a sample of compact polypropylene sheet, results similar to those described in Example 22 are obtained.

The following examples illustrate that embodiment of the present invention wherein the dyestuff is used as a dispersion.

### EXAMPLE 24

A sample of polypropylene fiber is impregnated (using a Foulard apparatus) in an aqueous bath at 50-60° C. containing a dispersion of 25 g./l. of solid Brilliant green

Romantrene (C.I. 59825) having a particle size less than 1 micron, dispersed into the bath with 25 g./l. of an anionic dispersing agent (the sodium salt of the dinaphthyl-methane-disulfonic acid).

- 5 The impregnated material is treated for 1 to 10 minutes in a suitable apparatus (a continuous polymerization reactor heated by hot air at 120-125° C.), with an aqueous bath containing sodium hydroxide and sodium hydrosulfite, at 50-60° C., keeping the pH between 9.5 and 10 by gradual addition of ammonium acetate, until the reduction of the vat dyestuff has been effected, is rinsed with cold water, soaped for 20-30 minutes with a solution at its boiling temperature, this solution containing the sodium salt of oleyl-methyl-taurinic acid and a suitable oxidizing agent (1-2 cc./l. of 30% hydrogen peroxide), rinsed, and dried.

The fiber is dyed green with a good uniformity at an intensity of 1/1 according to the standard ECE scale, and shows good general fastness and a fastness to natural light of at least one point on 8 higher than that when dyeing the same fiber using the same dyestuff reduced in a bath at 50° and pH 9.5-10.

### EXAMPLE 25

- 25 This example is similar to Example 24, but there was added to the impregnating bath suitable amounts of additives, to facilitate penetration and levelling of the dyestuff, e.g., from 2-70 g./l. of diethyl tartrate, and thickening agents compatible with the bath, e.g., Nafka rubber, 5-30 g./l. In this instance, 36 g./l. of diethyl tartrate was used, along with 18 g./l. of Nafka rubber. The fiber is dyed green and shows similar characteristics to those obtained by working according to the method described in Example 24, however with a higher uniformity, a higher purity, and brighter shade.

### EXAMPLES 26-35

- 40 By operating as described in Example 24, using each of the dyestuffs reported in Table 2, results and advantages similar to those described in Example 24 are obtained:

Table 2

| Example Number | Dyestuff                       | Color Index | Shade   |
|----------------|--------------------------------|-------------|---------|
| 26             | Yellow Romantrene GCN          | C.I. 67300  | Yellow. |
| 27             | Brilliant green Romantrene FEG | C.I. 59830  | Green.  |
| 28             | Brown Romantrene FR            | C.I. 69015  | Brown.  |
| 29             | Brown Romantrene FBR           | C.I. 70800  | Do.     |
| 30             | Yellow Romantrene F3RT         | C.I. 70805  | Yellow. |
| 31             | Olive Romantrene FR            | C.I. 69005  | Olive.  |
| 32             | Blue Romantrene FRS            | C.I. 69800  | Blue.   |
| 33             | Blue Romantrene FGD            | C.I. 69810  | Do.     |
| 34             | Blue Romantrene FBC            | C.I. 69825  | Do.     |
| 35             | Dark blue Romantrene FBO       | C.I. 59800  | Do.     |

### EXAMPLE 36

- 60 By operating as described in Example 25, but using each of the dyestuffs reported in Table 2, results similar to those of Example 25 are obtained.

### EXAMPLE 37

- 65 By operating according to each of Examples 24-36, using each of the dyestuffs of Table 2 on a sample of a compact polypropylene sheet and polyethylene sheet, results are obtained which are similar to those reported for the respective examples.

- 70
- 75
- EXAMPLE 38
- On a polypropylene fabric a printing is performed using a paste prepared according to Example 25, but using higher amounts of thickening agent (5 to 30 g./100 cc.).

The material thus printed is treated for 6 minutes at 120-125° C., cooled and impregnated in a Foulard apparatus with an alkaline solution of a thickened reducing agent (10 g. of starch as thickening agent, 15 g. sulfoxylate formaldehyde, 15 g. potassium carbonate, 60 g. water), treated for 6 minutes at a temperature not higher than 125° C., rinsed, soaped at the boiling temperature, rinsed again and dried.

Printing fabric is obtained which has a good degree of penetration, uniformity, and which has a fastness similar to those of the articles dyed in Example 25.

#### EXAMPLE 38

By operating as described in Example 37, using the dyestuffs reported in Table 2, similar results are obtained.

#### EXAMPLE 39

By operating as described in Example 37, but using the dyestuffs reported in Table 2 on a sample of a compact polypropylene sheet, similar results are obtained.

Variations can of course be made without departing from the spirit of this invention.

Having thus described the invention, what is desired to be secured and claimed by Letters Patent is:

1. A method for the dyeing and printing of a vat dyestuff on a shaped article of polypropylene, this method comprising:

- (a) impregnating said polypropylene with a treating material selected from the group consisting of a solution of a vat dyestuff in alkaline leuco form and a dispersion of a vat dyestuff;
- (b) removing the impregnated polypropylene from said treating material and heating said impregnated polypropylene at a temperature of from about 120 to 125° C.,
- (c) where a dispersion of a vat dyestuff is used in said impregnating step (a), reducing the dyestuff present in the heat treated, impregnated polypropylene to the alkaline leuco form, and
- (d) soaping said impregnated polypropylene with a soap solution at its boiling temperature while contemporaneously oxidizing said dyestuff.

2. A method for dyeing and printing of vat dyestuffs on polypropylene a shaped article of material comprising:

- (a) impregnating the polypropylene material with a solution of a vat dyestuff in alkaline leuco form,
- (b) removing the impregnated polypropylene from said treating material and heat treating the impregnated polypropylene material at a temperature of from about 120 to 125° C., and
- (c) soaping said impregnated polypropylene with a soap solution at its boiling temperature while con-

45

5

temporaneously oxidizing said dyestuff to thereby oxidize the dyestuff directly while it is on the polypropylene material.

3. The method of claim 1 wherein the oxidizing is effected using a hydrogen peroxide solution having a volume concentration of about 30% hydrogen peroxide.

4. The method of claim 1 wherein the vat dyestuff is selected from the group consisting of anthraquinone dyestuffs, indigo dyestuffs, thioindigo dyestuffs, carbazole dyestuffs, benzanethrone dyestuffs, and anthranthrone dyestuffs.

5. A shaped article of polypropylene dyed according to the method of claim 2.

6. The method of claim 2 wherein said impregnation of said polypropylene with a vat dyestuff in leuco form is carried out in the presence of an additive selected from the group consisting of the sodium salt of ligninsulfonic acid, the sodium salt of naphthalene sulfonic acid, the sodium salt of dinaphthylmethane-disulfonic acid, and diethyl tartrate.

7. A method for dyeing and printing of vat dyestuff in the dispersed state on a shaped article of polypropylene comprising:

- (a) impregnating the polypropylene material with a dispersion of a vat dyestuff,
- (b) removing the impregnated polypropylene from said treating material and heat treating the impregnated polypropylene material at a temperature of from about 120 to 125° C.,
- (c) reducing the dyestuff to the alkaline leuco form while on the polypropylene material, and
- (d) oxidizing the dyestuff and contemporaneously soaping the impregnated polypropylene using a soap solution at its boiling temperature.

8. A shaped article of polypropylene dyed according to the method of claim 7.

9. The method of claim 7 wherein said impregnation of said polypropylene with a vat dyestuff in leuco form is carried out in the presence of an additive selected from the group consisting of the sodium salt of ligninsulfonic acid, the sodium salt of naphthalene sulfonic acid, the sodium salt of dinaphthylmethane-disulfonic acid, and diethyl tartrate.

#### References Cited by the Examiner

##### UNITED STATES PATENTS

|           |         |              |      |
|-----------|---------|--------------|------|
| 2,774,647 | 12/1956 | Mecco et al. | 8-34 |
| 2,829,118 | 4/1958  | Wehr.        |      |
| 3,056,643 | 10/1962 | Kutner       | 8-55 |
| 3,122,409 | 2/1964  | Bardt        | 8-55 |

NORMAN G. TORCHIN, Primary Examiner.

UNITED STATES PATENT OFFICE  
CERTIFICATE OF CORRECTION

Patent No. 3,233,960

February 8, 1966

Bruno Lonardo

It is hereby certified that error appears in the above numbered patent requiring correction and that the said Letters Patent should read as corrected below.

Column 3, lines 30 and 31, for "oleyl-methyl-turinic" read -- oleyl-methyl-taurinic --; column 4, line 17, for "to be known" read -- to known --; lines 68 and 69, for "dyestug reduced" read -- dyestuff reduced --; column 6, line 75, for "agent) 5 to 30" read -- agent (5 to 30 --; column 7, line 44, strike out "on polypropylene a shaped article of" and insert instead -- on a shaped article of polypropylene --; column 8, line 21, for "printing of vat dyestuff" read -- printing of vat dyestuffs --.

Signed and sealed this 7th day of February 1967.  
**SEAL)**

**Attest:**

**ERNEST W. SWIDER**  
Attesting Officer

**EDWARD J. BRENNER**  
Commissioner of Patents